

## UNITED STATES PATENT OFFICE

2,691,001

## MINERAL LUBRICATING OIL COMPOSITION

Elmer B. Cyphers, Cranford, and David W. Young,  
Westfield, N. J., assignors to Standard Oil De-  
velopment Company, a corporation of Delaware

No Drawing. Application July 23, 1952,  
Serial No. 300,492

2 Claims. (Cl. 252—52)

1

The present invention relates to the use of 4,4' isopropylidene bis (2-isopropylphenol) as an additive for mineral lubricating oil compositions.

Various bis phenols have been suggested as additives for organic compositions subject to oxidation. The use of such phenols containing a bis linkage in the para position with respect to the hydroxyl radicals has met with little success. For example, diphenyol propane is relatively ineffective as a lubricant antioxidant. Furthermore, this compound cannot be used in the usual mineral lubricant compositions because it is substantially completely insoluble in such materials at ordinary temperatures.

In accordance with the present invention it has been found that mineral lubricating oil compositions containing dissolved therein small amounts of 4,4' isopropylidene bis (2-isopropylphenol) are excellent compositions for use in lubricating internal combustion engines and the like. Moreover, this particular bis phenol is soluble in oxidation inhibiting quantities over a wide range of temperatures. This specific compound also has unexpected advantages as an inhibitor over diphenyol propane and over analogous bisphenols in which the bis linkage is in the ortho position with respect to the hydroxyl groups.

The bis phenol of the present invention has the following structure:



This compound is readily and inexpensively prepared by condensing ortho isopropylphenol with propionaldehyde or dimethyl ketone, usually in the presence of a condensation catalyst. The general method of preparation of such compounds is well known to the art and does not form a part of the present invention.

The 4,4' isopropylidene bis (2-isopropylphenol) is dissolved in mineral lubricating oils in amounts in the range of about 0.05 to 1.5 or 2% by weight, the upper limit being restricted to some extent by the type of mineral oil base stock being used. A preferred concentration is in the range of about 0.1 to 1.0% by weight.

The lubricating oil base stocks used in the compositions of this invention may be straight mineral lubricating oils or distillates derived from paraffinic, naphthenic, asphaltic or mixed base crudes. The lubricating base stocks will generally range from about 40 to 150 seconds (Say-

2

bolt) viscosity at 210° F. The viscosity index may range from about 0 to 100 or higher, although for aviation lubricants, which are the preferred base stocks in the practice of the present invention, the higher viscosity indexes are preferred. The bisphenol of the present invention is quite suitable, however, for automotive lubricants, diesel lubricants and the like. In addition to the above mentioned materials, compositions may contain other agents including pour point depressants, viscosity index improvers, oiliness agents and the like.

The invention will be more fully understood by reference to the following examples. These examples, however, are given for the purpose of illustration only and are not to be construed as limiting the scope of the present invention in any way.

## Example 1.—Solubility studies

The bis phenol compound of the present invention, 4,4'-isopropylidene bis (2-isopropylphenol) was found to be readily soluble in mineral lubricating oils to the extent of as much as 1.0 to 1.5 weight percent at room temperature.

Diphenyol propane, on the other hand, was insoluble in mineral lubricants at room temperature. A solution was obtained when 0.25 weight percent diphenyol propane was agitated in a mineral lubricant at a temperature of 250° F., but, on cooling to room temperature, this bisphenol substantially completely crystallized out of solution.

## Example 2.—Staeger oxidation studies

Two highly solvent-extracted Mid-Continent lubricant base stocks were used in these studies. Base stock I had an S. S. U. viscosity at 210° F. of 85. Base stock II had an S. S. U. viscosity at 210° F. of 43 and a viscosity index of 112. Blends of each of these oils containing 0.25 weight percent of various bisphenols as well as the oils per se were tested.

The test employed was a modification of the Staeger test and consisted essentially of storing a 200 ml. sample of oil in a rotating shelf oven maintained at 100° C.  $\pm 1$ . A 40 x 70 mm. freshly polished copper strip was placed in the 400 ml. container to serve as an oxidation catalyst. The strip was removed every 72 hours and replaced by a clean strip. The shelf moved at an angular velocity of 4-6 R. P. M., and positive ventilation of 1.5 to 2.0 cubic feet of air per hour was maintained. Oil samples were withdrawn periodically from the container and the neutralization num-

ber determined. The oxidation life is defined as the time in hours required to obtain an increase in neutralization number of 0.20 mg. KOH/g.

When testing the blend containing diphenylol propane, it was necessary to heat the material when forming the solution and to keep the solution hot when transferring it to the test container.

The results are shown in the following table:

| Additive Tested                                             | "Staeger" Oxidation Life, Hours |               | 10 |
|-------------------------------------------------------------|---------------------------------|---------------|----|
|                                                             | Base Stock I                    | Base Stock II |    |
| None                                                        | 75                              | 95            |    |
| Diphenylol propane                                          | 75                              | 85            |    |
| 4,4'-isopropylidene-di-o-cresol                             | 84                              | 220           | 15 |
| 4,4'-isopropylidene bis (2-isopropylphenol)                 | 154                             | 440           |    |
| 2,2' bis (2-hydroxy-3-tert.-butyl-5-methoxy-phenyl) propane | 100                             | 285           | 20 |

The compound of the present invention is about two to four times as effective as the corresponding bisphenols containing either no alkyl substituents or methyl substituents. It is also markedly superior to a meta bisphenol containing methoxy substituents.

*Example 3.—Aluminum cup coking studies*

Oil blends were prepared containing various concentrations of several bisphenols in a solvent-extracted Mid-Continent aviation base oil having a viscosity at 210° F. of about 100 Saybolt seconds. These blends and a sample of the base oil per se were evaluated by the aluminum cup coking test. This test determines the effectiveness of an additive for inhibiting coking of lubricants under the severe temperature conditions normally encountered in aviation engines.

The test was conducted by placing the oil in an aluminum measuring cup of known weight and stirring the oil while applying heat. The side walls of the cup were maintained at a temperature of 500° F. while heating the oil at the bottom

until it reached 550° F. The stirring was then stopped for 10 minutes followed by stirring for 10 minutes. At the end of the fourth alternate stirring and non-stirring period, the oil was discarded, and the cup was weighed. The results are shown in the following table:

| Additive in Base Stock                                            | Aluminum Cup Deposits, Mg. Coke per 75 g. of Oil | 10   |                                                             |
|-------------------------------------------------------------------|--------------------------------------------------|------|-------------------------------------------------------------|
|                                                                   |                                                  | None | 0.5 wt. percent 4,4'-isopropylidene bis (2-isopropylphenol) |
| 0.5 wt. percent 2,2'-methylene bis (4-methyl-6-tert.-butylphenol) | 27                                               |      |                                                             |
| 1.0 wt. percent 2,2'-methylene bis (4-methyl-6-tert.-butylphenol) | 44                                               |      |                                                             |
|                                                                   | 25                                               |      |                                                             |

The compound of the present invention is considerably more effective than a related compound having a bis configuration ortho to the hydroxyl groups and alkyl substituent groups in both ortho and para positions.

What is claimed is:

1. A mineral lubricating oil composition containing a major proportion of a mineral lubricating oil and dissolved therein a minor oxidation inhibiting amount of 4,4'-isopropylidene bis (2-isopropylphenol).
2. A composition as in claim 1 wherein the amount of said bis phenol is in the range of about 0.05 to 1.5% by weight, based on the total composition.

References Cited in the file of this patent

UNITED STATES PATENTS

| Number    | Name      | Date           |
|-----------|-----------|----------------|
| 2,017,827 | Bannister | Oct. 5, 1935   |
| 2,295,985 | Baird     | Sept. 17, 1942 |
| 2,482,748 | Dietzler  | Sept. 27, 1949 |
| 2,515,906 | Stevens   | July 18, 1950  |
| 2,591,651 | Young     | Apr. 1, 1952   |
| 2,636,002 | Capelli   | Apr. 21, 1953  |
| 2,651,572 | Eichhoff  | Sept. 8, 1953  |